

Oct. 29, 1940.

A. J. NERAD

2,219,935

## MERCURY BOILER

Filed June 21, 1938

Fig. 1.



Fig. 2.



Inventor:  
Anthony J. Nerad

by Harry E. Dunham  
His Attorney.

## UNITED STATES PATENT OFFICE

2,219,935

## MERCURY BOILER

Anthony J. Nerad, Schenectady, N. Y., assignor  
to General Electric Company, a corporation of  
New York

Application June 21, 1938, Serial No. 214,987

28 Claims. (Cl. 122—318)

The present invention is a continuation in part of my application Serial No. 48,859, filed November 8, 1935, and relates to mercury boilers, generally to vessels made from ferrous metal for heating mercury in which the mercury comes into contact with the ferrous metal at high temperatures, for example, temperatures of the order of 1000° F. It has been found that mercury at high temperatures, especially at the operating temperatures of mercury boilers, causes dissolving of ferrous metal from which the boiler elements are made. Inhibitors such as aluminum, nickel, chromium, magnesium, and calcium have been discovered which, when added to the mercury, prevent or reduce to a considerable extent the dissolving of ferrous metal by mercury at the operating temperature of mercury boilers. Arrangements and methods of operating mercury boilers of this type are more fully disclosed in my Patent 1,964,593, filed July 1, 1933, and assigned to the same assignee as the present application.

Another difficulty met with in the operation of mercury boilers is due to the fact that mercury ordinarily does not wet ferrous metal. I have found that wetting of the ferrous metal boiler walls by mercury liquid may be accomplished by the adding of certain agents such as sodium or potassium. An arrangement and a method of operating mercury boilers of this kind is covered by my Patent 1,964,592, filed August 17, 1931, and assigned to the same assignee as the present application.

Certain inhibitors may form a thick coating on the ferrous metal surfaces in contact with the mercury. Such heavy coatings are undesirable, particularly when formed in very narrow channels through which the mercury flows because the thick coating may lead to plugging of such channels. A further difficulty experienced in the operation of mercury boilers is the formation of heavy lumps caused by the oxidation of certain ingredients such as sodium when added to the mercury. Such lumps may endanger the operation of a mercury boiler by plugging fluid passages. There always will be oxidation of agents but the oxides thus formed which constitute waste should not be in the form of lumps but rather in a powdery form which does not interfere with the flow of mercury through the heating elements.

One object of the present invention is to provide an improved arrangement and method of operating a mercury boiler of the type specified above, whereby the dissolving of ferrous metal

by the mercury at high temperatures is prevented, and satisfactory wetting of the boiler walls by the mercury liquid is attained.

Another object of my invention is to provide an improved method of and arrangement for adding inhibitors and wetting agents or substances to the mercury, whereby the protective and wetting effect of such agents is initiated within a short period of time.

Other objects of my invention are the provision of inhibitors and agents for mercury boilers which do not cause plugging of passages by the formation of very thick coatings or lumps of oxides.

For a consideration of further objects and features of my invention, attention is directed to the following description and the claims appended thereto in connection with the accompanying drawing.

In the drawing, Fig. 1 is a somewhat diagrammatic view of a mercury boiler embodying my invention, and Fig. 2 is a detail of Fig. 1.

In the course of extensive tests and research work on mercury boilers, I have discovered certain substances which, when added to the mercury in sufficient amounts, prevent substantially completely the dissolving of ferrous metal by the mercury at the operating temperature of the boiler, which at the present time is of the order of 1000° F. Two of these substances which have given very satisfactory results are zirconium and titanium. These substances act primarily as inhibitors, reducing the dissolving of ferrous metal by the mercury, but they also act as wetting agents when added to the mercury in sufficient amounts. The use of these substances has distinct advantages. They form, when added to the mercury, extremely thin layers or coatings on or with the ferrous metal walls of the boiler. These layers or coatings adhere to the boiler surface. They may also partly penetrate into the surface and form alloys with ferrous metal of the boiler walls. The thickness of these coatings is not increased substantially by the addition of excessive amounts of these substances. This is important in mercury boiler arrangements including a number of heating elements forming narrow passages because layers of considerable thickness formed in these passages by excessive amounts of such substances would considerably reduce the flow of fluid therethrough, and in certain cases might cause clogging thereof. Thus, the use of these substances not only inhibits the dissolving of ferrous metal, but also assures the formation of a reasonably uniform layer of extreme thinness of

- good heat conductivity, and consequently a uniform flow of fluid through the various elements of the boiler. Another distinct advantage of zirconium and titanium is that they do not form bulky or voluminous oxides or ferrites which reduce the danger of clogging of the narrow and small diameter passages by the inhibitors themselves. The oxidation products of zirconium and titanium in mercury boilers form powdery, dry substances which may be readily removed from the boiler by means of sumps, traps, or the like. One of the most outstanding characteristics of zirconium and titanium, when used as inhibitors, is their effectiveness in very small amounts.
- 15 Titanium and zirconium are only slightly soluble in mercury at boiler temperatures. By way of comparison, it has been found that roughly from 10,000 to 100,000 times more aluminum can be held in solution at temperatures from 1000 to 20 1200° F. than zirconium or titanium. This fact is important in that it prevents extreme concentration at any point in the boiler; or from another viewpoint, it assures more uniform distribution of the inhibitors throughout the different 25 elements of the boiler. Due to the low solubility of zirconium and titanium in mercury, coatings formed on the mercury boiler walls resist redisolution more than other known inhibitors and the presence of this coating together with the 30 metal in the mercury results in the complete protective action.

Zirconium and titanium added to mercury boilers as pure metals are present during any or all of the following states: (a) In solution in the 35 hot mercury in small amounts; (b) Deposited as an extremely thin and uniform coating on or alloyed with the mercury-wetted boiler surfaces; and (c) In the form of well wetted, finely divided particles. When the boiler is cooled down then, 40 due to the fact that these metals are so slightly soluble in the mercury at low temperatures, most of the dissolved metal crystallizes out of the mercury in the form of very fine particles and these particles are well wetted. This is of decided advantage because such wetted crystallized particles 45 are not as susceptible to attack by oxygen which may leak into the boiler during shut down periods (as single molecules in a dissolved state). In contrast hereto, other inhibitors, such as aluminum, which are more soluble in mercury, combine with oxygen much more readily than either titanium or zirconium because such other inhibitors are in molecular state rather than in the 50 form of wetted particles protected by a coating of mercury. Mercury containing zirconium and titanium in amounts sufficient to completely protect a boiler from the dissolving action of the mercury has been kept for days in bottles with air over the mercury without causing serious oxidation of these inhibitors. The reliability and the 55 economy of a mercury boiler are considerably improved by the adding of one of these inhibitors to the mercury.

As stated above, either of the elements of the 60 group zirconium and titanium in addition to their effect as inhibitors act as de-oxidizing agents in a mercury boiler. I have found that the de-oxidizing action of these substances, however, may reduce to some extent their inhibiting effect, particularly when used in systems in which considerable amount of oxygen is present. Also the coating on the boiler walls formed by zirconium and titanium may become oxidized in the presence of oxygen and such oxidized coating reduces 65 the heat transfer from the wall to the mercury.

because the latter does not properly wet the oxidized coating. I have found that these difficulties are overcome by adding to the mercury together with an inhibitor a de-oxidizing agent which has an affinity to oxygen stronger than that of the inhibitor. If zirconium or titanium are used as inhibitors, I have found that aluminum, magnesium and calcium when added to such inhibitor act as strong de-oxidizing agents. Ordinarily these substances, aluminum, magnesium and calcium, act as inhibitors when used alone, that is, prevent the mercury from dissolving ferrous metal walls at high temperatures. The use of magnesium or calcium as de-oxidizing agent is preferable because neither forms a coating on the boiler walls when used together with zirconium or titanium.

The use of strong de-oxidizing agents, such as magnesium and calcium, in mercury boilers increases the economy of the process. These 20 agents reduce oxides in the system, in particular oxides formed by zirconium and titanium. Hence, the entire amount of zirconium or titanium added to the mercury is maintained in an effective state in which such substances form coatings and thereby inhibit the dissolving action of mercury at high temperatures on ferrous metal. The oxides of zirconium and titanium being ineffective as inhibitors, it is desirable to maintain such inhibiting substances in a metallic state. Thus, 30 with the addition of strong de-oxidizing agents, the waste of inhibitors due to oxidation is avoided. Practically complete stoppage of dissolving of ferrous metal by mercury has been accomplished with an amount of inhibitor equal to one 35 part by weight in 100,000 parts of mercury. In cases in which the oxidizing agents, such as sodium, are used to effect wetting of the boiler surfaces by the mercury, the addition of magnesium or calcium has the advantage that either of these 40 substances reduces oxides formed by sodium or the like and thereby breaks up large lumps of sodium oxides to form a powder, thus preventing the plugging of fluid passages.

Only comparatively small amounts of zirconium or titanium are needed for complete boiler protection. For instance, in a large commercial mercury vapor boiler installation of more than 50 30,000 square feet boiler surface in which zirconium is used, complete protection against dissolving of ferrous metal is obtained over a two month period of operation with three parts by weight of zirconium in 10,000 parts of mercury. This particular system is known to have contained substantial quantities of metal oxides and the system also is subject to infiltration of oxygen 55 during operation.

Summarizing, complete protection of a mercury boiler may be obtained by adding to the mercury one of the elements of the group zirconium and titanium and one of the elements of the group magnesium and calcium. The addition of these substances inhibits the dissolving of ferrous metal, causes wetting of the boiler surfaces by the mercury and reduces oxides in the 60 boiler into harmless and readily removable dry powders. Such complete protection over a long period of time may be attained by periodic tests and the addition of such substances whenever needed. To this end samples of boiler fluid are 65 taken from the boiler during operation and chemically analyzed to determine the amount of inhibiting and de-oxidizing substances in the mercury. Such analysis may be made daily, depending upon the conditions of the boiler. Satis- 70 75

factory results have been obtained by maintaining concentration of zirconium metal in the mercury above .0002% by weight and of magnesium above .001% by weight. It is preferable to maintain the concentration of magnesium within the range of .001% to .01% by weight and of the inhibitors within the range of .0002% to .002%. The periodic analysis of the boiler fluid is especially important in boiler systems which are intermittently operated and which are subject to air infiltration. Whenever these analyses show a deficiency of either the inhibiting or reducing substance, the necessary amount of such substances are added to make up the deficiency.

15 The protective action or effect of titanium or zirconium is complete as soon as the inhibitor is uniformly distributed throughout the boiler system and has formed a coating on or with the ferrous metal walls. The time lag between the 20 adding of these substances or inhibitors and their complete effectiveness or protective actions, that is, the formation of a coating on or with the boiler walls, is reduced in accordance with an improved method of adding these substances. Before describing the method itself, attention is directed to the fact that zirconium and titanium in their commercial form are not chemically pure, but include certain impurities, and what is more important, they are covered with a thin layer of 25 oxide. If added in this form directly to the mercury in a mercury boiler, it obviously takes a certain period of time until the oxide film is broken down or removed from the particles and the elements are wetted by the mercury. This 30 undesirable time lag is reduced in accordance with my invention by prewetting the substances to be added to the mercury boiler by means of mercury liquid. It is also known that non-wetted particles are carried out of the boiler with 35 the vapor whereas wetted particles are not carried out except in mercury liquid mechanically suspended in the mercury vapor, such suspended liquid being negligible in the system and may be substantially eliminated by the provision of 40 known liquid vapor separating means. For the purpose of prewetting, zirconium or titanium are put into a hermetically sealed container or bomb together with a certain amount of mercury and heated therein in the absence of air to prevent 45 oxidation of the metals. Heating of the mixture is necessary to effect wetting of the substances by the mercury. This prewetting may be accelerated if the substance such as zirconium or titanium is added to the mercury as powder. As 50 stated before, titanium and zirconium have a low solubility in mercury. By adding these elements in the form of powder to mercury liquid large surfaces, as compared to the weight or volume of these elements, are contacted by the 55 mercury. This is important also when titanium and zirconium are added in nonwetted form directly to the mercury boiler because it limits the possibility of clogging the narrow and small diameter passages and permits rapid wetting of the 60 substances by the mercury.

65 The prewetting of zirconium and titanium by mercury may be further accelerated by stirring the mixture of mercury and zirconium or titanium. As to the relative amounts of mercury and zirconium for prewetting the zirconium, it has been found desirable to use an amount of mercury sufficient to maintain fluidity of the mixture. Satisfactory results have been obtained by mixing 18 to 54 parts by weight of mercury with 70 1 part by weight of zirconium or titanium at a

temperature of the order of about 1000° F. To exclude air or oxygen during the prewetting, the mixture is preferably placed in a hermetically sealed bomb, and to accelerate the wetting process, the bomb is preferably moved, tilted, or oscillated in a rocking furnace for a period of 50 to 100 hours to make sure that the particles are well wetted.

A further important feature of my invention is the provision of means for and a method of protecting a mixture of mercury and wetted zirconium or like substance against oxidation and the consequent de-wetting of the substance, especially when these are highly concentrated. I have found that this may be accomplished by adding to the mixture of mercury and titanium or like substance a small amount of zinc, copper, or like film stabilizing agent. A piece or particle of zirconium or titanium is prewetted, when its surface has been brought into intimate contact with the mercury. The mercury then has a strong tendency to adhere to such surface. A prewetted surface is ordinarily rapidly de-wetted when such particle is exposed to oxygen or air. The de-wetting of a wetted particle is considerably reduced by the provision of a film stabilizing substance in the mercury. As said before, a particle is wetted when a film of mercury adheres strongly to the surface of the particle. Such film of mercury may be stabilized by a small amount of zinc or copper so that a wetted particle may be exposed to air for a considerable period of time. The surface film toughening substance may be added to the mercury during the prewetting process. Satisfactory results have been obtained with mixtures comprising about 18 parts by weight of mercury, 1 part of titanium and  $\frac{1}{6}$  part of zinc. Such mixture is preferably sealed in a low carbon steel tube or bomb and heated at 1000° F. for about 50 to 100 hours in a rocking furnace. The tubes are kept sealed until the mixture is to be added to a mercury boiler. Often the prewetted powder lumps together. These lumps may be easily broken up by stirring to form a homogeneous and fluid substance before being supplied to the boiler.

In arrangements in which a strong de-oxidizing agent, such as magnesium or calcium, is to be used in the boiler, together with zirconium or titanium, the mixture of mercury and wetted zirconium may be protected against oxidation by adding to it either magnesium or calcium. In this case I have obtained good results by loading a bomb with 18 to 54 parts by weight of mercury to one part of titanium or zirconium with a small amount of magnesium or calcium. In such case a stabilizing substance, such as zinc or copper, may be dispensed with, provided great care is taken in supplying the mixture contained in the bomb to the boiler. The great affinity of magnesium or calcium for oxygen allows this process to be carried out in ordinary low carbon steel bombs at a temperature of the order of 900° F.

The arrangement illustrated in the drawing comprises a drum 10 of ferrous metal covered by lagging or like heat insulating material 11 held in place by a cover 12. The drum is partly filled with mercury liquid 13 to which has been added an inhibitor or substance as hereinbefore described. A filler block 14 is provided in the liquid space of the drum for displacing a portion of the liquid to minimize the amount of liquid necessary for operating the boiler. Fastened to the lower portion of the drum 10 are a plurality of heating tubes 15 made from ferrous metal. Each

heating tube (Fig. 2) comprises an outer tubular member 16 fastened to the wall 10 of the drum, and a core or inner tubular member 17 having an inner wall 18 and an outer wall 19 welded together 5 to define a hermetically closed space. The inner wall 18 defines a passage 20 communicating at its lower end with a passage 21 defined between the outer wall 19 and the outer tube 16. A sleeve 22 is fastened at its upper end to a baffle plate 23 disposed within the drum 10 and with its lower end extends into the passage 20 defined by the inner wall of the core. During operation, mercury liquid is conducted from the space above a baffle plate 23 in the drum 10 through the sleeve 22 into 10 the passage 20, whence it flows into the passage 21 defined between the outer tube 16 and the outer wall 19. Heat is conducted to the tubes and the drums by radiation and conduction. The liquid contained in the outer passage 21 is partly 15 evaporated and conducted to the drum. The provision of a double-walled core in the tube minimizes the direct heat transfer from the outer passage 21, which may be termed the vapor passage, into the inner passage 20 which may be termed the liquid passage. This results in a differential pressure between the fluids conducted through the two passages, to the effect that a steady flow or circulation of fluid through said passages takes place. The vapor produced in the boiler is conducted 20 through a conduit 24 to a turbine 25, whence the exhaust is received by a condenser 26 having cooling means 28. The condensate is returned to the drum by means of a conduit 29 connected to the condenser 26 and a pipe 30 between the conduit 25 25 and the drum 10.

Besides the drums 10 and the heating tubes connected thereto, other heating units or elements may be provided. In the present instance I have shown a heating unit 31 having a header 32 communicating with the liquid in the drum through a conduit 33. The heating unit 31 comprises a down-tube 34 connecting the header 32 to a lower header 35, located external a wall 36 of the furnace. The lower header 35 is connected to the lower ends of up-tubes 37 located inside the wall 36 of the furnace and having their upper ends projecting through the furnace wall and connected to the upper header 32. The tubes 37 form a wall screen for the furnace wall 36.

50 During operation, mercury liquid contained in the tubes 37 is heated to form vapor. The fluid in these tubes rises and flows into the upper header 32. The vapor thus formed is conducted through the conduit 33 to the drum and the liquid 55 is recirculated through the down-tubes 34 and the up-tubes 37. To prevent the up-stream from the tubes 37 from interfering with the liquid flowing into tubes 34, a baffle plate 38 is provided in the upper header 32.

60 The arrangement for adding inhibiting and wetting substances in accordance with my invention comprises a standpipe 40 connected at the lower end to an intermediate point of the down-tube 34. The standpipe includes a lower valve 65 41 and an upper valve 42 and has an upper portion formed to define a funnel 43. A substance may be added to the boiler during operation by first opening the valve 42, then pouring the substance into the pipe 40, thereafter closing the valve 42, and finally opening the valve 41 to permit the substance to flow into the down-tube 34 to be carried into the boiler system. To prevent large pieces from being supplied into the boiler, a strainer 44 is provided at the lower end of the 70 75 funnel 43.

Zirconium and titanium, when added in the form of powder, have a tendency to float on the surface of the mercury, and difficulties have been experienced in forcing these substances into the system due to their light weight. These difficulties are overcome by the provision of a tank 45 for containing mercury liquid 46 connected to the funnel 43 by a conduit 47 including a valve 48. During the adding of powdered titanium, zirconium or like substance, the valve 48 is opened 10 together with the valve 42, so that the substance is flushed into the tube 40 by a stream of mercury liquid discharged from the tank 46. The mercury is preferably supplied from the tank 46 in dry form. Water is separated from the mercury 15 by the provision of heating means, in the present instance a steam coil 49 disposed within the tank 46.

The system also includes means permitting the removal of boiler fluid for analysis to assure the 20 presence of an efficient amount of inhibiting and oxygen-reducing substances in the active state. This means has been shown in the drawing as comprising a pipe 50 connected to down-tube 34 and including two valves 51 and 52 arranged in 25 series. With this arrangement, boiler fluid may be removed during operation by opening the valve 51 to permit boiler fluid to flow into the portion of the pipe 50 between the valves 51 and 52. Thereafter the valve 51 is closed and the valve 30 52 opened.

Every possible precaution should be taken to eliminate conditions allowing contact between the inhibitors and oxygen or oxides in order to have at all times in the mercury these inhibitors 35 in metallic state in the boiler. All parts of the system must be carefully sealed. Preferably nitrogen or other inert gas is leaked into the system during shut-down periods.

While I have described my invention particularly in connection with mercury boilers, it is not limited thereto necessarily but may be utilized wherever conditions are met with which make it desirable to overcome the tendency for mercury to dissolve ferrous metal at high 40 temperatures.

In accordance with the provisions of the patent statutes, I have described the principle of operation of my invention, together with a particular method and apparatus which I now consider to 50 represent the best embodiment thereof, but I desire to have it understood that the particular method and apparatus disclosed are only illustrative, and that the invention may be carried out with such modifications as come within the scope 55 of the appended claims.

What I claim as new and desire to secure by Letters Patent of the United States is:

1. A mercury boiler having ferrous metal tubes through which mercury circulates between a 60 region of higher temperature and a region of lower temperature, said boiler being charged with mercury to which has been added an inhibitor which forms an extremely thin coating on the tube surface contacting the mercury together with a de-oxidizing agent which has stronger affinity to oxygen than the inhibitor.

2. A mercury boiler having ferrous metal tubes through which mercury circulates between a 70 region of higher temperature and a region of lower temperature, said boiler being charged with mercury to which has been added an inhibitor and a de-oxidizing agent, the inhibitor including a metal which has very low solubility in mercury and at the operating temperature of the boiler 75

forms an extremely thin uniform coating on the boiler surfaces contacting the mercury, and the de-oxidizing agent having an affinity to oxygen stronger than that of the inhibitor.

5. 3. A mercury boiler having ferrous metal tubes through which mercury circulates between a region of higher temperature and a region of lower temperature, said boiler being charged with mercury to which has been added an element of the group titanium and zirconium.

4. A mercury boiler having ferrous metal tubes through which mercury circulates between a region of higher temperature and a region of lower temperature, said boiler being charged with mercury to which has been added an element of the group titanium and zirconium together with a de-oxidizing agent with greater affinity to oxygen than either element of said group.

5. A mercury boiler having ferrous metal tubes through which mercury circulates between a region of higher temperature and a region of lower temperature, said boiler being charged with mercury to which has been added an element of the group titanium and zirconium together with at least one element of the group magnesium and calcium.

6. A mercury boiler having ferrous metal tubes through which mercury circulates at high temperature, said boiler being charged with mercury to which has been added an element of the group titanium and zirconium of an amount of more than .0001% by weight of mercury.

7. A mercury boiler having ferrous metal tubes through which mercury circulates at high temperature, said boiler being charged with mercury to which has been added an element of the group titanium and zirconium in an amount of the order of .0002% by weight of the mercury together with an amount of an element of the group magnesium and calcium of the order of more than .001% by weight of mercury.

8. An operating fluid for containers having ferrous metal walls subject to high temperatures during operation comprising mercury and a small amount of a substance associated with the mercury which substance forms an extremely thin coating on ferrous metal when contacted by the fluid at high temperature, and a small amount of a reducing agent to prevent oxidation of said substance and to reduce oxides when added to the container.

9. A composition for operating boilers having ferrous metal walls comprising substantially entirely mercury and a small amount of a substance forming a thin dissolution resistant layer on ferrous metal at high temperature and a small amount of one of the elements of the group magnesium and calcium.

10. A mercury boiler including the combination of a container made from ferrous metal, mercury liquid contained in the container, and means to prevent dissolving of ferrous metal by the mercury at the operating temperature of the boiler and to effect wetting of the boiler surfaces by the mercury liquid, said means comprising one of the elements of the group zirconium and titanium in the mercury liquid of an amount of about .04% by weight of the mercury.

11. A mercury boiler including the combination of a container made from ferrous metal, mercury liquid contained in the container, means to prevent dissolving of ferrous metal by the mercury at the operating temperature of the boiler and to effect wetting of the boiler surfaces by the mercury liquid, said means comprising one of the ele-

ments of the group zirconium and titanium in the mercury liquid, and means to maintain the concentration of such element above .0001% by weight of the mercury.

12. A mercury boiler including the combination of a container made from ferrous metal, mercury liquid contained in the container, means to prevent dissolving of ferrous metal by the mercury at the operating temperature of the boiler and to effect wetting of the boiler surfaces by the mercury liquid, said means comprising one of the elements of the group zirconium and titanium in the mercury liquid, and means including a valved conduit connected to the boiler for supplying one of said elements to the boiler during operation thereof to maintain the concentration of such element above .0001% by weight of the mercury and one of the elements of the group magnesium and calcium in the mercury liquid.

13. In the operation of a mercury boiler having ferrous metal walls, the method of adding to the mercury an inhibitor in powdered form and the adding of one of the elements of the group magnesium and calcium to prevent oxidation of the inhibitor.

14. In the operation of a mercury boiler having ferrous metal tubes through which mercury liquid is circulated during operation, the method of adding to the mercury a mixture in powdered form, which mixture includes an element of the group titanium and zirconium and an element of the group calcium and magnesium.

15. A substance for protecting mercury containers made from ferrous metal against dissolving of the ferrous metal by the mercury at high temperature, such substance including a pretreated mixture of a small amount of an inhibitor and a comparatively large amount of mercury together with a reducing agent to prevent oxidation of the inhibitor.

16. The method of preparing a working fluid for a mercury boiler having ferrous metal tubes with surfaces contacted by heated mercury during operation, which method comprises mixing a small amount of an inhibitor which is wetted by mercury when heated with a comparatively large amount of mercury liquid, heating the mixture in the absence of oxygen to cause the mercury to wet the inhibitor and thereafter adding the mixture to the mercury in the boiler.

17. The method of preparing a working fluid for a mercury boiler having ferrous metal tubes with surfaces contacted by heated mercury during operation, which method comprises mixing a small amount of one of the elements of the group zirconium and titanium with a large amount of mercury, and heating the mixture in a hermetically sealed vessel to effect wetting of the element by the mercury.

18. The method of preparing a working fluid for a mercury boiler having ferrous metal tubes with surfaces contacted by heated mercury during operation, which method comprises mixing powder of one of the elements of the group titanium and zirconium with mercury liquid, agitating the mixture, heating the mixture during agitation in the absence of oxygen, and supplying the mixture to the liquid in the boiler.

19. The method of preparing a working fluid for a mercury boiler having ferrous metal tubes with surfaces contacted by heated mercury during operation, which method comprises mixing an inhibitor which is wetted by mercury when heated with mercury liquid and a small amount of an element of the group zinc and copper,

- heating the mixture and supplying it to the mercury in the boiler.
20. The method of preparing a working fluid for a mercury boiler having ferrous metal tubes with surfaces contacted by heated mercury during operation, which method comprises mixing an inhibitor with a reducing agent of greater affinity to oxygen than the inhibitor, heating the mixture and supplying it to the mercury liquid in the boiler.
21. The method of preparing a working fluid for a mercury boiler having ferrous metal tubes with surfaces contacted by heated mercury during operation, which method comprises mixing an element of the group zirconium and titanium with at least one element of the group zinc, copper, magnesium and calcium and a comparatively large amount of mercury liquid, and supplying the mixture to the liquid in the boiler.
22. The method of preparing a working fluid for a mercury boiler having ferrous metal tubes with surfaces contacted by heated mercury during operation, which method comprises mixing an element of the group zirconium and titanium and an element of the group magnesium and calcium with a large amount of mercury liquid, heating the mixture at a temperature of the order of 900° F. and supplying the mixture to the mercury liquid in the boiler.
23. A ferrous metal container through which mercury liquid is circulated at high temperature, said container being charged with mercury, an element of the group zirconium and titanium and a strong oxygen-reducing agent.
24. A mercury boiler having tubes made from ferrous metal through which mercury liquid is circulated at high temperature, said boiler being charged with an inhibitor which is wetted by mercury when heated to form a thin coating on the boiler walls to prevent dissolving thereof by the action of mercury at high temperature and an excess of inhibitor to maintain the coating and a small amount of one of the elements of the group zinc and copper to stabilize the protective layer formed on the ferrous metal and thereby render it more resistant against the destructive action of oxygen.
25. A substance for protecting mercury boilers having heating elements made from ferrous metal against the dissolving action of mercury on the ferrous metal at high temperature, which substance includes about eighteen parts of mercury, one part of an element of the group zirconium and titanium and a fraction of one part of an element of the group zinc and copper, 10 magnesium and calcium.
26. A mercury boiler comprising tubes made from ferrous metal through which mercury is circulated during operation, and means for conducting inhibiting and oxygen reducing substances into the tubes during operation of the boiler, said means including a standpipe connected to one of the tubes and including lower and upper valve means.
27. A mercury boiler comprising tubes made from ferrous metal through which mercury is circulated during operation, means for conducting a substance into the tubes during operation of the boiler, said means including a standpipe connected at its lower end to one of the tubes, 25 a lower and upper valve in the standpipe, a funnel secured to the upper end of the standpipe, and a sieve intermediate the funnel and the upper valve to prevent large solid pieces from being conducted into the standpipe.
28. A mercury boiler having heating units made from ferrous metal for heating and operating mercury liquid, said units including down tubes disposed outside the boiler, and means for conducting an inhibitor into the heating units 35 during operation, said means including a standpipe having a lower end connected to an intermediate portion of the down tube, a lower and upper valve in the standpipe, a funnel secured to the upper end of the standpipe, and means for flushing solid inhibitors from the funnel into the standpipe, said last-named means comprising a container for liquid mercury connected to the upper end of the standpipe, and means for drying mercury liquid in the container.

ANTHONY J. NERAD.